

## UNITED STATES PATENT OFFICE

2,614,983

METHOD OF PREVENTION OF CORROSION  
IN WELLSJoseph A. Caldwell and Melba L. Lytle, Houston,  
Tex., assignors, by mesne assignments, to  
Standard Oil Development Company, Eliza-  
beth, N. J., a corporation of DelawareNo Drawing. Application April 3, 1950,  
Serial No. 153,770

5 Claims. (Cl. 252—8.55)

1

The present invention is directed to a method for inhibiting the corrosiveness to corrodible metal surfaces of corrosive subsurface fluids containing carbon dioxide. More particularly, the invention relates to a method for inhibiting the corrosivity of corrosive well fluids containing carbon dioxide to corrodible ferrous metal conduits and attendant equipment through which the fluids are flowed and processed.

In many oil fields and gas-condensate fields, the production of fluids from subsurface formations is accompanied by extremely severe corrosion of the conduits and attendant equipment which is contacted by the fluid mixture being produced. In many cases it is found that the fluid mixture is acidic in nature and contains substantial amounts of carbon dioxide, a portion of which dissolves in water or brine present in the fluids to form carbonic acid. These fluids, including the carbon dioxide, originate in the subsurface formations. In some cases the corrosion occurs throughout the conduits and attendant equipment through which the fluids are flowed and processed while in other cases the corrosion is limited primarily to rather restricted areas of the conduit and is often particularly severe in that portion of the conduit adjacent the well head. If corrosion, whether intensive or extensive, is permitted to continue unabated, the conduit and attendant equipment will become sufficiently damaged to require replacement. Not only is the actual cost of such replacement high, but other factors may be involved which further increase costs. For example, it may be necessary to kill a high pressure well in order to make the necessary replacements. Furthermore, while replacements and repairs are being made, there is a loss in revenues due to having the well off production. Even of more importance than the high costs incurred as a result of corrosion is the danger that a well will flow wild as a result of the failure of the conduit or equipment due to corrosion. Such a result may be catastrophic.

It is therefore the main object of the present invention to provide a method whereby the corrosivity of corrosive well fluids containing carbon dioxide is substantially eliminated or inhibited in the conduits and attendant equipment through which the fluids from subsurface formations are flowed and processed.

In accordance with the present invention the corrosivity to corrodible ferrous metal surfaces by corrosive well fluids including moisture and carbon dioxide is eliminated or substantially re-

duced by incorporating in the corrosive fluids a corrosion inhibiting amount of fatty derivatives of polyethylene glycols. The lower molecular weight polyethylene glycols do not yield fatty derivatives which have practical effectiveness in inhibiting corrosion of ferrous metal surfaces by well fluids containing moisture and carbon dioxide. For example, the fatty derivatives of mono-, di-, tri-ethylene glycols are either completely ineffective or must be used in prohibitive quantities to effect substantial inhibition. The most generally suitable and powerful fatty derivatives of polyethylene glycols are derived from polyethylene glycols of the type formula  $(OC_2H_4)_x(CH_2OH)_2$  in which C designates carbon, H designates hydrogen, O designates oxygen, and X has a value of from 3 to 30. It is preferred to employ a polyethylene glycol in which the value of X in the foregoing formula is in the range of 6 to 15. The  $(OC_2H_4)_x$  group in the foregoing formula will hereinafter be designated by the term "ethoxy" group. Fatty derivatives prepared from nonaethylene glycol, for example, are particularly effective. Other polyethylene glycols which may be mentioned by way of example include: tetraethylene glycol, pentaethylene glycol, hexaethylene glycol, heptaethylene glycol, octaethylene glycol, decaethylene glycol, dodecaethylene glycol, tri-decaethylene glycol, pentadecaethylene glycol, etc.

The fatty material employed to produce the fatty derivatives of polyethylene glycol may be selected from the class of fatty acids and fatty oils. Acids having from 12 to 26 carbon atoms per molecule such as palmitoleic, oleic, ricinoleic, linoleic, linolenic, licanic, arachidonic, clupanodonic, lauric, myristic, arachidic, stearic, palmitic, etc. and fatty oils from which such acids can be derived may be reacted with the polyethylene glycols to produce the desired corrosion inhibiting agents. Especially effective agents are obtained by reacting the polyethylene glycols with such fatty oils as linseed oil, cottonseed oil, tung oil, oiticica oil, China-wood oil, castor oil, menhaden oil, and the like, or mixtures thereof. Likewise, mixtures of polyethylene glycols may be employed. In any event, the fatty material selected is reacted with the polyethylene glycol selected at a temperature in the range of from 300° to 550° F. for a time in the range of from 1 to 5 hours in the presence of a small amount of an alkaline reacting catalyst such as an alkali hydroxide or carbonate or mixtures thereof. The fatty derivatives of

polyethylene glycols prepared in the foregoing manner are soluble in many aromatic solvents and, to a more limited extent, in petroleum solvents such as heavy naphtha or kerosene.

The polyethylene glycols which are employed in the preparation of the fatty derivatives of the present invention are readily available. They may be made, for example, by reacting ethylene oxide with water, the formation of polyethylene glycols being favored by maintaining the molal ratio of ethylene oxide to water in excess of 1. The degree of polymerization is further determined by the reaction conditions maintained. Polyethylene glycols having molecular weights in excess of 1500 are commercially available as well as polyethylene glycols having lower molecular weights. For use in the preparation of the fatty derivatives employed in accordance with the present invention, it is not necessary that the polyethylene glycols be separated into close fractions of narrow molecular weight limits; on the contrary, fractions including a large number of polymers of different molecular weights may be employed.

When fatty derivatives of the present invention are prepared from a fatty oil, it is preferable that the fatty oil be present in the initial reaction mixture in a weight ratio of from about 1:1 to about 3:1 as compared to the polyethylene glycol. When the fatty derivative is prepared from a fatty acid, the fatty acid should be present in the initial reaction mixture in a weight ratio of from about 0.5:1 to about 2:1 as compared to the polyethylene glycol. Only a small amount of the alkaline reaction catalyst need be present, and ordinarily 3 weight per cent or less of the catalyst based on the weight of the reaction mixture is necessary. For example, a concentration of about 1% by weight of sodium hydroxide based upon the weight of the reactants has been found sufficient to promote the reaction. On the other hand, as little as about 0.5 weight per cent of sodium hydroxide based on the weight of the reactants has been found sufficient when from about 0.5 weight per cent to about 2 weight per cent of sodium carbonate is utilized as a co-catalyst. In another instance 0.05 weight per cent of sodium hydroxide gave good results.

The amount of fatty derivatives of the present invention employed to inhibit the corrosion of ferrous metal surfaces by gas-condensate well fluid mixtures including moisture and carbon dioxide may be varied over a relatively wide range although it has been found that amounts within the range of 0.005 per cent to 0.1 per cent by volume of the fluid mixture gives satisfactory results. Ordinarily, however, an amount within the range of 0.005 to 0.01 per cent by volume will give satisfactory inhibition.

Inasmuch as the fatty derivatives of the present invention are soluble in certain solvents, examples of which have been heretofore mentioned, it may be found convenient to dissolve the fatty derivative in a suitable solvent before introducing it into the corrosive fluid mixture. When it is desired to protect from corrosion the conduit in the borehole, as well as the attendant equipment, the fatty derivative or a solution thereof may be injected into the borehole adjacent the subsurface formation from which the corrosive fluid, including carbon dioxide, is produced. Alternatively, the fatty derivative may be introduced directly into the conduit. A still further method of introducing the fatty deriva-

tive into the fluids produced from the subsurface formation involves introducing the fatty derivative or a solution thereof into the annular space between the casing and the tubing.

5 Another method of introducing the fatty derivative into the subsurface fluid consists of injecting the fatty derivative or a solution thereof into the subsurface reservoir through an adjacent well. Irrespective of the particular procedure employed in introducing the fatty derivative into the fluids in the well, the fatty derivative suppresses the corrosivity of the fluids, thereby eliminating or reducing damage to the conduit, through which the fluids are produced and to attendant equipment through which the fluids are flowed.

In order to determine the effectiveness of the fatty derivatives of polyethylene glycol employed in accordance with the present invention, a 20 derivative was prepared by reacting Chinese tung oil and nonaethylene glycol. This derivative was prepared in the following manner: 60 grams of Chinese tung oil, 40 grams of nonaethylene glycol, and 0.5 gram of sodium carbonate were 25 heated together at a temperature of 500°-550° F. for 2 hours. The reaction product thus formed was added to a 50:50 mixture of condensate and water obtained from a well located in the gas-condensate field at Katy, Texas, the reaction 30 product being added to the fluid mixture in a concentration of 0.01 per cent by volume. 100 cc. of the foregoing mixture was placed in each of two glass tubes and a mild steel coupon suspended therein. The fluid mixture in the tube 35 was then saturated with carbon dioxide and the tube sealed off. The coupon was immersed in the fluid mixture 31 times per minute for 14 days. Three other glass tubes containing 100 cc. of the brine-condensate mixture containing no inhibitor 40 were similarly tested as a control. The results obtained are shown in the table below:

Table

| Concentration of Inhibitor | Corrosion Rate of Coupons, Metal Loss, In./Yr. |        |        |         | Percent Reduction Over Blank |
|----------------------------|------------------------------------------------|--------|--------|---------|------------------------------|
|                            | A                                              | B      | C      | Average |                              |
| None                       | 0.0055                                         | 0.0049 | 0.0058 | 0.0054  | -----                        |
| 0.01 Vol. Percent          | 0.0003                                         | 0.0004 | -----  | 0.0004  | .95                          |

It will be noted that the corrosivity of the aforementioned well fluid to corrodible ferrous metal was substantially eliminated by the addition of a very small amount of the reaction product of tung oil and nonaethylene glycol.

The objects and advantages of the present invention having been fully described and illustrated, what we wish to claim as new and useful 60 and to secure by Letters Patent is:

1. A method for reducing the corrosiveness to corrodible ferrous metal of a corrosive well fluid including moisture and carbon dioxide which comprises introducing into said fluid a corrosion 65 inhibiting amount of a reaction product obtained by reacting a fatty material selected from the group consisting of fatty acids having at least 12 and no more than 26 carbon atoms per molecule and fatty oils containing fatty acid radicals having no less than 12 and no more than 26 carbon atoms with a polyethylene glycol containing at least 3 and no more than 30 ethoxy groups in the presence of an alkaline reacting catalyst selected from the group consisting of 70 alkali metal hydroxide and alkali metal carbon 75

for a period of time in the range of 1 to 5 hours at a temperature in the range of 300° to 550° F., the weight ratio of fatty material to polyethylene glycol being in the range of 1:1 to about 3:1.

2. A method in accordance with claim 1 in which the reaction product is added to the corrosive fluid in an amount in the range of 0.005 to 0.1 per cent by volume of the fluid.

3. A method for reducing the corrosiveness to corrodible ferrous metal of a corrosive petrolierous well fluid including moisture and carbon dioxide which comprises introducing into said fluid a corrosion inhibiting amount in the range of 0.005 to 0.1 per cent by volume of the fluid of a reaction product obtained by reacting tung oil with nonaethylene glycol in the presence of an alkaline reacting catalyst selected from the group consisting of alkali metal hydroxide and alkali metal carbon for a period of time in the range of 1 to 5 hours at a temperature in the range of 300° to 550° F., the weight ratio of tung oil to nonaethylene glycol being in the range of 1:1 to about 3:1.

4. A method for reducing the corrosiveness to corrodible ferrous metal of a corrosive petrolierous well fluid including moisture and carbon dioxide which comprises introducing into said fluid a corrosion inhibiting amount in the range of 0.005% to 0.1% by volume of the fluid of a fatty derivative obtained by reacting cottonseed oil with nonaethylene glycol in the presence of an alkaline reaction catalyst selected from the group consisting of alkali metal hydroxide and alkali metal carbonate for a period of time in

the range of 1 to 5 hours at a temperature in the range of 300° to 550° F., the weight ratio of cottonseed oil to nonaethylene glycol being in the range of 1:1 to about 3:1.

5. A method for reducing the corrosiveness to corrodible ferrous metal of a corrosive petrolierous well fluid including moisture and carbon dioxide which comprises introducing into said fluid a corrosion inhibiting amount in the range of 0.005 to 0.1 per cent by volume of the fluid of a fatty derivative obtained by reacting oiticica oil with nonaethylene glycol in the presence of an alkaline reacting catalyst selected from the group consisting of alkali metal hydroxide and alkali metal carbon for a period of time in the range of 1 to 5 hours at a temperature in the range of 300° to 550° F., the weight ratio of oiticica oil to nonaethylene glycol being in the range of 1:1 to about 3:1.

20 JOSEPH A. CALDWELL.  
MELBA L. LYTHE.

#### REFERENCES CITED

The following references are of record in the file of this patent:

#### UNITED STATES PATENTS

| Number    | Name   | Date          |
|-----------|--------|---------------|
| 2,249,800 | Weber  | July 22, 1941 |
| 2,460,259 | Kahler | Jan. 25, 1949 |
| 2,527,889 | Moore  | Oct. 31, 1950 |

#### OTHER REFERENCES

Ind. & Eng. Chem., vol. 40, No. 12, p. 2344.  
35 Article by Baker et al.